

## UNITED STATES PATENT OFFICE

1,920,212

## METHOD OF MANUFACTURING ARTIFICIAL THREADS OR FILAMENTS

Reginald William Payne and Robert Pierce Roberts, Spondon near Derby, England, assignees to Celanese Corporation of America, a Corporation of Delaware

No Drawing. Original application December 12, 1928, Serial No. 325,480, and in Great Britain December 23, 1927. Divided and this application February 27, 1930. Serial No. 431,965

## 4 Claims. (Cl. 18—54.)

This invention relates to the manufacture of artificial filaments or threads from solutions of cellulose acetate or other esters or ethers of cellulose by the dry spinning or evaporative method of formation and is a division of application Serial No. 325,480, filed December 12, 1928.

In the spinning of such artificial threads or filaments by the dry spinning or evaporative method of formation, solutions of cellulose acetate or other esters or ethers of cellulose in volatile solvents are spun into an evaporative atmosphere (usually into a current of heated air) the threads or filaments so formed being continuously wound up, with or without twisting, on apparatus situated within or outside the evaporative atmosphere. The threads or filaments heretofore produced by such method of spinning have been lustrous in character and have found successful application as artificial silk, artificial horse hair and the like.

The object of the present invention is to produce threads or filaments presenting reduced lustre and more particularly threads or filaments presenting a dull, matt or lustreless appearance, or of considerably reduced lustre.

For this purpose, according to the invention, we employ solutions of cellulose derivatives in volatile solvents and containing one or more organic precipitants for the cellulose derivative and we perform the spinning of said solutions by the dry or evaporative method under such conditions that the organic precipitant or precipitants exert a precipitating action on the filaments in the natal state of the filaments.

In performing the invention we may extrude said solutions into evaporative atmospheres such as air or into evaporative atmospheres containing one or more of the organic precipitants.

In performing the invention we may employ as the precipitant any organic substance or substances capable of precipitating the cellulose ester or ether from its solution in the volatile solvent employed. Thus, for instance, we may employ alcohols (for instance, ethyl alcohol, cyclohexanol), hydrocarbons (e. g. benzene, xylene, petrol, petroleum ether), or esters (e. g. butyl propionate), or ethers (e. g. propyl ether), but it will of course be understood that the choice of precipitant will depend upon the solubility characteristics of the cellulose ester or ether employed and on the relative boiling points of the volatile solvents and precipitants.

According to one form of execution of the invention we may extrude into a heated metier casing or spinning cell, through which a current

of air is caused to pass, a solution of cellulose acetate or other ester or ether of cellulose containing one or more of the precipitants. In such form of execution the quantity of precipitant will vary according to its boiling point and its precipitating power on the solution of the cellulose ester or ether employed and with the spinning conditions and the result it is desired to achieve. In general, quantities of precipitant of from about 1% or less to 40% or more, and preferably from about 5% to 30%, relatively to the volatile solvent should be employed in this form of execution, but it will be understood that these quantities are only given by way of illustration. The quantities of precipitant employed should of course be sufficient to cause a precipitation of the cellulose derivatives from solution under the conditions of spinning.

The following example illustrates a form of execution of the invention.

## Example

Highly satisfactory threads or yarns presenting reduced lustre may be produced by extruding any of the following solutions into an evaporative atmosphere of air heated to a temperature between 40° and 80° C., for instance, downwards into a suitably heated metier casing or spinning cell (such for instance as described in U. S. Patents Nos. 1,602,125, 1,541,104 and 1,731,317) through which a current of air is caused to pass in an upward or downward direction.

## Solution A

|                        | Parts | 90 |
|------------------------|-------|----|
| Acetone (99-100% pure) | 100   |    |
| Xylene                 | 20    |    |
| Cellulose acetate      | 40    |    |

## Solution B

|                        | Parts | 95 |
|------------------------|-------|----|
| Acetone (99-100% pure) | 100   |    |
| Butyl propionate       | 20    |    |
| Cellulose acetate      | 40    |    |

## Solution C

|                        | Parts | 100 |
|------------------------|-------|-----|
| Acetone (99-100% pure) | 97    |     |
| Xylene                 | 23    |     |
| Cellulose acetate      | 40    |     |

## Solution D

|                        | Parts | 105 |
|------------------------|-------|-----|
| Acetone (99-100% pure) | 103   |     |
| Xylene                 | 17    |     |
| Cellulose acetate      | 40    |     |

By varying the temperature of the heated air

the above solutions will yield filaments showing varying degrees of delustration. Thus with air at a temperature of 40° C. the filaments are substantially completely delustrated and are of dull or matt appearance, and the degree of delustration decreases as the temperature of the air is raised. With air at a temperature of 80° C. the filaments are slightly delustrated, and have a highly satisfactory medium low lustre.

10 It is to be understood that these solutions are given only by way of example and are in no way limitative.

15 In performing the invention we preferably wind the filaments or threads up (continuously with their formation) with or without twisting, on apparatus located outside the evaporative atmosphere, though such winding may be performed within said atmosphere if so desired.

20 It is to be understood that the invention is in no way limited to the particular examples of execution described, which may be varied widely.

25 The filaments may be extruded either downwards or upwards into the spinning cell or metier casing, and the air current (which may be caused to pass either downwards or upwards through the metier casing or cell) may be heated or warmed therein or prior to admission thereto or both before and during passage through the cell or metier casing. Further, the filaments may be extruded in the same direction as or counter-current to the air current.

30 The temperatures to be employed in the spinning cells or metier casings may vary with the boiling point of the solvents and precipitants used, the composition of the spinning solutions and the degree of delustration it is desired to produce in the filaments or threads. Such temperatures may be higher or lower than the boiling point or points of the solvent or solvents employed.

35 We have found that with spinning solutions containing the more usual solvents such as acetone, methyl acetate or the like, temperatures of about 40° to 80° C. may usefully be employed in

the spinning cells or metier casings but we in no way limit ourselves to such temperatures.

40 By means of the present invention it is possible to obtain threads or filaments showing any desired degree of reduced lustre, from a completely delustrated or matt appearance to a relatively high lustre, according to the proportion of precipitant present and the spinning conditions employed.

45 What we claim and desire to secure by Letters Patent is:—

50 1. Process for the production of artificial filaments presenting reduced lustre characterized in that solutions of cellulose esters in volatile solvents and containing xylene are spun by the dry or evaporative method of formation under such conditions that the xylene exerts a precipitating action on the filaments in the natal state of the filaments.

55 2. Process for the production of artificial filaments presenting reduced lustre characterized in that solutions of cellulose acetate in volatile solvents and containing xylene are spun by the dry or evaporative method of formation under such conditions that the xylene exerts a precipitating action on the filaments in the natal state of the filaments.

60 3. Method of producing artificial filaments presenting reduced lustre which comprises extruding into a current of air heated to a temperature of between 40° and 80° C. a solution of cellulose acetate composed of 97 parts acetone, 23 parts xylene, and 40 parts cellulose acetate.

65 4. Method of producing artificial filaments presenting reduced lustre which comprises extruding downwards through orifices into a spinning cell a solution of cellulose acetate composed of 97 parts acetone, 23 parts xylene and 40 parts cellulose acetate, and causing a current of air heated to a temperature between 40° and 80° C. to pass upwards through said cell.

70 REGINALD WILLIAM PAYNE.  
ROBERT PIERCE ROBERTS.

120

45

125

50

130

55

135

60

140

65

145

70

150

75